

# UNITED STATES PATENT OFFICE.

ARTHUR SCHLEGEL, OF MANNHEIM, GERMANY, AND KARL PFISTER, OF PHILADELPHIA, PENNSYLVANIA, ASSIGNORS TO BADISCHE ANILIN & SODA FABRIK, OF LUDWIGSHAFEN-ON-THE-RHINE, GERMANY, A CORPORATION.

## PROCESS FOR PRODUCING STABLE DYEINGS.

1,121,295.

Specification of Letters Patent.

Patented Dec. 15, 1914.

No Drawing.

Application filed December 4, 1913. Serial No. 804,721.

*To all whom it may concern:*

Be it known that we, ARTHUR SCHLEGEL and KARL PFISTER, citizens of the German Empire, residing, respectively, at Mannheim, 5 Germany, and Philadelphia, State of Pennsylvania, have invented new and useful Improvements in Processes for Producing Stable Dyeings, of which the following is a specification.

10 In the specification of Patent No. 893,384 one of us has described and claimed a process of dyeing with vat coloring matters of the anthracene series by applying a paste of the said coloring matters to the fiber and 15 then treating the material with an alkaline reducing agent in the presence of water and alkali. For this purpose the textile material, after bleaching or extracting with boiling water, was treated with a paste of the coloring matter either by padding or printing, and the material was then either dried or 20 rolled up without being dried. In a subsequent operation the material was treated, after having been so prepared, with a solution or suspension of an alkaline reducing agent. In the application of the coloring matter it could be used with or without the 25 addition of a thickening agent. When operating as described in the example of the 30 said Patent No. 893,384 it is directed that the cotton should be treated in the alkaline reducing bath for about 30 minutes, that is to say, the material is allowed to pass forward and backward through the bath, for 35 instance in a jigger.

We have now invented an improved method of carrying out the said process, whereby it is not necessary to treat the material for such a long time in the reducing bath, a 40 sufficient fixation of the dyestuff being attained by a single passage of the material, to which the coloring matter has been applied, for a very short time through an alkaline reducing bath which, however, in this 45 case must be much more concentrated with regard to hydrosulfite. In this way, the dyer is in a position to arrange the two steps, namely the application of the dyestuff to the material and the passage through the reducing bath, in a continuous manner and to 50 carry out the whole process easily and in a shorter space of time and thus to produce more dyed material in a given time.

The new process is carried out as follows.

A suspension of the coloring matter, or mixture of coloring matters, which may contain a thickening agent, or may contain caustic soda, or both, is applied to the goods in a padding machine, the squeezing rollers of which are so arranged that the material absorbs about 80% of its weight of the dye suspension. After one single treatment as described, the material (either without being dried or rolled up, or after having been dried and rolled up, or dried without being rolled up) is passed into the developing solution which consists of a warm strong hydrosulfite solution containing caustic alkali. After a short single passage through this liquid, the material is rolled up on a suitable roller. The reduction of the coloring matter and its fixation on the fiber becomes completed while the material is on this roller. These operations can be carried out in an ordinary jigger in which a small trough provided with a roller is inserted to hold the hydrosulfite solution. For ordinary working, this trough need not contain more than 2 gallons of solution and as the material removes the solution from the trough, a sufficient fresh quantity is continuously added.

By way of example, we give the following quantities that can be applied in carrying out this invention, but the invention is not confined to this example.

For dyeing about 110 lbs. of cotton cloth, that is to say 12 pieces, prepare a thin paste from about 27 lbs. of a vat coloring matter which can be obtained according to United States Letters Patent No. 753,659, and known in commerce as indanthrene blue GCD, 1 lb. 5 oz. of a vat coloring matter such as can be obtained according to United States Letters Patent No. 856,811, known in commerce as indanthrene Golden Orange G, 95 2 lbs. of caustic soda and 24 gallons of water. Pass the goods through this paste once as above described, keeping the coloring matter suspended in the liquid uniformly by stirring. A thickening agent may also be added to assist in the maintenance of a uniform suspension. During this treatment, the material should absorb about 11 gallons of the suspension. The alkaline reducing bath is prepared from 6 to 8 lbs. of commercial sodium hydrosulfite, 4.5 lbs. of caustic soda and 21 gallons of water. This solution should have a temperature of about 160° F.

in the tank in which it is stored, so that its temperature in the trough in which it is applied to the material is about 140° F. The goods are passed once through this solution as described and absorb about 11.5 gallons of the liquid.

Now what we claim is:—

The process for producing stable dyeings by passing the material to be dyed through 10 a paste of a vat coloring matter of the anthracene series and then fixing the coloring matter on the fiber by a single short passage through a warm alkaline hydrosulfite solution containing about three to four parts

of sodium hydrosulfite per hundred parts 15 of water.

In testimony whereof we have hereunto set our hands in the presence of two subscribing witnesses.

ARTHUR SCHLEGEL.  
KARL PFISTER.

Witnesses to the signature of Arthur Schlegel:

J. ALEC. LLOYD,  
S. S. BERGER.

Witnesses to the signature of Karl Pfister:  
HUGO HILL,  
CARL RICKHARDT.